

April 29, 1941.

J. H. TAYLOR

2,240,319

METHOD OF PRODUCING PIPE FITTINGS

Filed July 24, 1939

2 Sheets-Sheet 1

Fig. 1.



Fig. 2.



Fig. 3.



Inventor  
James Hall Taylor

By Brown, Jackson, Buttler & Vining  
Atty's. of

April 29, 1941.

J. H. TAYLOR

2,240,319

METHOD OF PRODUCING PIPE FITTINGS

Filed July 24, 1939

2 Sheets-Sheet 2

FIG. 4.



FIG. 5.



FIG. 6.



Inventor  
James Hall Taylor

By Brown, Jackson, Cuttler, Vienna  
Atty. U.S. & Co.

## UNITED STATES PATENT OFFICE

2,240,319

## METHOD OF PRODUCING PIPE FITTINGS

James Hall Taylor, Oak Park, Ill.

Application July 24, 1939, Serial No. 286,136

4 Claims. (CL. 29—157)

This invention relates to the manufacture of wrought metal pipe fittings of the nature of T's, having a trunk or body provided with an extension or neck substantially perpendicular to the trunk, and has to do with an improved method and improved apparatus for producing such fittings.

It is known to produce a T by reducing the end portions of a tubular blank and thereby producing a protuberance at one side of the blank, and then form the protuberance to provide the neck of the T. In such known method, however, the wall of the neck of the T is of the same thickness as the wall of the body or trunk of the T. The neck opening through the trunk weakens the wall of the latter and if a T, produced by the known method referred to, be subjected to interior bursting pressure it will burst at the base of the neck, which is the weakest portion of the structure. In order to avoid that difficulty it is the usual practice to form T's, when produced in accordance with the known method referred to, from blanks having a wall thickness appreciably greater than the wall thickness of the pipe with which the T is to be used, the wall thickness of such blanks being referred to as of greater than standard thickness, the wall thickness of the pipe to which the T is to be applied being considered as standard. That is objectionable as necessitating the use in the production of the T of a greater amount of metal than would be necessary if the T were produced from a blank of standard wall thickness, that is, of the same wall thickness as the pipe to which the T is to be applied.

In my Patent No. 1,892,712, issued January 3, 1933, I have disclosed a method of producing a T, in the manner above stated, in which patent outward extensions or skirts are produced at the end portions of the trunk of the T, it being necessary to move such skirts and end portions of the T trunk in finishing the T. The removed metal is waste, which is objectionable for obvious reasons. While the method of my patent referred to possesses certain advantages and is efficient in certain respects, I find that that method can be improved upon by eliminating the waste of metal referred to.

The instant invention is directed primarily to the production of T's and analogous pipe fittings from tubular blanks of standard wall thickness, that is, of the same wall thickness as the pipe to which the T is to be applied, and to the reduction of waste metal to a minimum, to the end of reduced cost in the production of T's and analogous fittings. More specifically, I reduce the end por-

tions of a tubular blank, of standard wall thickness, from one side thereof and thereby displace and redistribute metal at the middle portion of that side in such manner that the wall and the base portion of the neck of the T is materially thickened and thereby reinforced, to such an extent that the area of the T at the base of the neck is at least as strong as the remaining portions of the T. In accomplishing the results referred to, I employ certain novel apparatus, effective for displacing and redistributing the metal of the blank in the manner referred to, as will be explained more fully hereinafter. Further objects and advantages of my invention will appear from the detail description.

In the drawings:

Figure 1 is a central lengthwise sectional view through a tubular blank from which the T of my invention is to be produced;

Figure 2 is a central sectional view through the blank of Figure 1 with an end portion thereof formed between cooperating inner and outer dies, shown in elevation and in section, respectively, illustrating the first step of my method;

Figure 3 is a sectional view through a pair of exterior dies and a blank formed thereby over an interior die, shown in elevation, illustrating the second step of my method;

Figure 4 is a central lengthwise sectional view through the partially formed blank of Figure 3 disposed over an interior die, shown in elevation, and a pair of opposed exterior dies, shown in section, illustrating the third step of my invention;

Figure 5 is a view similar to Figure 4 illustrating a continuation of the step shown in the latter figure; and

Figure 6 is a central lengthwise sectional view through a T produced by my method.

In producing a T in accordance with the method of my invention, I start with a wrought metal tubular blank *b* such as that shown in Figure 1. A substantially semi-elliptical area *7* of this blank, at one end portion thereof, is heated in a suitable manner to a proper working temperature such that the metal of that area, when subjected to pressure, will readily flow. The blank *b*, with the area *7* thereof heated as stated, is then placed upon an interior die *8* fixedly mounted in a suitable manner and provided with a collar *9* against which the other end of the blank seats. Die *8* comprises a cylindrical body *10* extending from collar *9* and having its other end portion *11* of reduced diameter, with a shoulder *12* extending between the portions *10* and *11* and inclined at

such an angle that the metal of portion 7 of the blank, when subjected to pressure, will readily flow upward along the shoulder. I find that having shoulder 12 at an inclination of approximately 30° to portion 11 of die 8 produces satisfactory results. The interior die 8 cooperates with an exterior die 13 having a cylindrical bore 14 extending from its outer end, this bore being of a radius greater than the radius of portion 11 of die 8 by an amount equal to the thickness of the wall of blank  $b$ . This blank is of standard wall thickness, that is, of the same wall thickness as the pipe to which the T to be produced is to be applied. Outer die 13 is further provided, at one side thereof, with a recess 15 similar in shape to shoulder 12 of die 8, the inner end of this recess merging into a bore 16 extending from the inner end of die 13 and of the same diameter as the exterior of blank  $b$ .

After blank  $b$ , with the area 7 thereof heated as stated, has been placed over the interior die 8, exterior die 13 is moved toward die 8, in the direction of the arrow  $a$ , into the position shown in Figure 2. In the latter figure the position of the end portion of blank  $b$  extending about shoulder 12 and portion 11 of die 8, when the blank is disposed upon the latter die and preliminary to inward movement of die 13, is indicated, in part, by the dot and dash lines. In the inward movement of die 13 the upper side portion of blank  $b$  is reduced and the shoulder of the recess 15 of die 13 subjects that portion of the blank to combine radial and lengthwise inward pressure. The metal from portion 7 of the blank is thus displaced by a combined upsetting and scraping action and is redistributed in such manner as to provide a thickened wall element 17 extending from the upper side of the reduced end portion of the blank to the central unreduced portion of the blank. The thickening of the metal at element 17 is provided for by having the shoulder 12 and the wall of recess 15 of die 13 so related as to define a space of maximum width or thickness adjacent the reduced end portion of the blank and tapering toward such portion and toward the unreduced central portion of the blank, as will be clear from Figure 2. During the inward movement of die 13 the shoulder of recess 15 of that die may exert a scraping and upsetting effect on the metal sufficient to move the upper portion of the end of the blank inward a short distance. The end of the reduced portion of the blank then is beveled or inclined as shown in Figure 2. In the latter figure the inclination of the end of the reduced portion of the blank is exaggerated for purposes of illustration. In practice such beveling or inclination of the end of the blank due to reduction thereof may, in many cases, be very slight and, in some cases, may not occur to any appreciable extent. After the blank of Figure 1 has had its end portion reduced and shaped by means of the die 13 cooperating with the interior die 8, it becomes the partially formed blank  $b^1$  of Figure 2. In the latter blank the thickened element 17 and the adjacent unreduced central portion of the blank form a projection at one side thereof.

Blank  $b^1$  is then removed from the interior die 8 and is placed over an interior cylindrical die 18 corresponding in diameter to the interior diameter of the reduced end portion of blank  $b^1$ , the end of this reduced portion of the blank being first trimmed, if inclined, so as to be normal to the axis of the blank, and seating against a stop collar 19 at one end of die 18, the latter die being

fixedly mounted in a suitable manner. This reduced end portion of the blank is also inserted into an exterior die 20, seating against collar 19, the latter die having a recess 21 conforming to the exterior surface of the thickened wall portion 17 of the blank, which recess merges into a cylindrical bore 22, of the same diameter as the exterior of the reduced end portion of the blank, and a cylindrical bore 23 of the same diameter as the exterior of the unreduced central portion of the blank. The reduced end portion of the blank, as well as the unreduced central portion thereof and the portion corresponding to the thickened wall element 17, is confined, by means of the exterior die 20 and the interior die 18, in such manner as effectively to prevent distortion thereof. When the blank  $b^1$  of Figure 2 is thus positioned between the dies 18 and 20, the unreduced end portion of this blank occupies the position indicated by dot and dash lines in Figure 3. An area of this unreduced end portion of the blank, corresponding to area 7 of Figure 1, is then heated to suitable working temperature, or this area may be heated to suitable working temperature before positioning the blank upon die 18. Thereafter an exterior die 24, substantially similar to die 13, is moved inward along the interior die 18, in the direction of the arrow  $a^1$ . During inward movement of die 24 the end portion of the blank remote from collar 19 is reduced from the same side thereof as the other end portion of the original blank, producing the thickened wall element 17 similar to the element 17 produced by the exterior die 13 and the interior die 8. It will be noted that the interior die 18 of Figure 3 is of uniform diameter. When the die 24 moves inward of interior die 18 lengthwise thereof, the other end portion of the blank is cold and is confined against distortion by the exterior die 20 and interior die 18, in the manner above stated. Consequently, during inward movement of die 24 the heated area of the corresponding end portion of the blank is subjected to inward endwise and radial pressure and the displaced metal flows along the path of least resistance, into and along the wall of the recess of die 24, so as to produce the thickened wall element 17 referred to. The two thickened wall elements 17 are connected, at their inner ends, by wall element 25 at the unreduced central portion of the blank, thus producing the blank of Figure 3, which may be designated  $b^2$ . The elements 17 and 25 together constitute a protuberance 26 at one side of the blank  $b^2$ , this blank comprising a body or trunk having the reduced end portions and the protuberance 26 between such end portions at one side of the blank.

The blank  $b^2$  is then provided with a suitable opening 27 through protuberance 26 centrally thereof, by punching or in any other suitable manner, producing the blank  $b^3$  of Figure 4. This blank is placed over an interior cylindrical die 28 of a diameter corresponding to the interior diameter of the reduced end portions of the blank. Die 28 is provided with a recess which receives a substantially frusto-spherical plug 29 having a maximum exterior diameter corresponding to the desired interior diameter of the neck of the T to be produced. Plug 29 is initially disposed within the circumference of die 28 and is positioned therewith within the blank  $b^3$ , the plug then being coaxial with opening 27 of protuberance 26. Suitably recessed upper and lower dies 30 and 31 are then closed about blank  $b^3$ , these exterior dies abutting, at one end, a stop

collar or flange 32 on die 28. Upper die 30 is provided with a cylindrical opening 33 of a diameter corresponding to the exterior diameter of the neck of the T, the inner or base portion of opening 33 being defined by a rounded fillet 34. 5 A pull rod 35 is then inserted through opening 27 and is secured to plug 29 centrally thereof, conveniently by screw means. Rod 35 is then pulled upward, as indicated by the arrow, raising plug 29 out of die 28 into contact with the inner face 10 of protuberance 26. In the continued upward movement of rod 35 and plug 29 protuberance 26 is bent upward and outward and is shaped conformably to the opening 33, as will be clear from Figure 5. This upward movement of the plug continues until the opening 27 has been expanded to a diameter equal to the maximum diameter of plug 29, which then passes upward through the neck thus produced. In this manner the protuberance 26 is shaped to provide the neck of the T, the upper end of which neck may be trimmed off, as may be the ends of the body or trunk of the T, if desired. The T in its finished form is shown in Figure 6. It will be noted that in the finished T the neck 26a is connected at its base 25 portion to the body or trunk of the T by fillets 17a of considerably greater wall thickness than the remainder of the T. These fillets effectively reinforce the T at the area of juncture between the neck and the trunk thereof, eliminating 30 danger of bursting of the T in that area. By thus reinforcing the base of the neck and the adjacent areas of the T, I render it practicable to produce the T from a blank of standard wall thickness, that is, of the same wall thickness as the pipe to 35 which the T is to be applied. That is advantageous as effecting saving in metal in the production of the T, since it eliminates necessity of using a blank of greater than standard wall thickness. Also, since in practice the inclination of 40 the ends of the blank, incident to reduction of the end portions thereof, may be slight or nonexistent, the necessity of trimming any considerable amount of metal from the blank or the T in the process of production thereof is eliminated, thus effecting a further saving in that respect.

In Figures 2 and 3 I have assumed, for purposes of description, that the dies 13 and 24 are the movable dies, the dies 9 and 19 being the fixed dies. That is not essential to the method of my invention, however, and either or both of the dies, in either case, may be moved endwise, it sufficing so long as the dies have relative endwise movement effective for accomplishing the results desired. I consider the shouldered die 8 of Figure 2, cooperating with the exterior die 13, of value as providing simple and efficient means whereby one end portion of the blank may be reduced preliminary to reduction of the other end portion 45 thereof, a shouldered interior die not being necessary to reduction of the other end portion of the blank, for the reasons above stated. Within the broader aspects of my invention, the reduction and shaping of the end portions and associated elements of the blank may be effected in any desired order by any other means suitable for that purpose. By properly heating both of the end portions of the blank b, placing it upon an interior die 18 of suitable length, and imparting 50 relative movement to dies 20 and 24 of Figure 3 lengthwise of die 18, one toward the other, the blank b<sup>2</sup> of Figure 3 may be produced from the blank b of Figure 1 in a single operation. While 55 that is satisfactory in many cases, I prefer, in 70 75

certain cases, to form the blank b<sup>2</sup> of Figure 3 in two operations, including the operation of Figure 2 employing the shouldered interior die 8 of the latter figure.

I claim:

1. The method of producing a T, which comprises heating selected areas at one side of the end portions of a tubular metal blank to such a temperature that the metal thereof will readily flow when subjected to pressure, subjecting such areas to combined inward radial and lengthwise pressure effective for reducing the end portions of the blank relative to the central portion thereof and for upsetting the wall of the blank at the 15 areas of juncture between the end portions and the central portion, thereby producing the trunk of the T and a protuberance at said one side of the trunk intermediate the end portions thereof with the wall of the base portion of the protuberance of greater thickness than that of the trunk, and forming the protuberance to final size and shape thereby producing the neck of the T joined to the trunk by a fillet of greater wall thickness than the trunk.

2. The method of producing a T, which comprises heating a selected area at one side of one end portion of a tubular metal blank to such a temperature that the metal thereof will readily flow when subjected to pressure, reducing said end portion relative to the central portion of the blank from said one side thereof by subjecting it to combined inward radial and lengthwise pressure between an interior shouldered die and an exterior recessed die effective for upsetting the wall of the blank at the area of juncture between the central portion and said reduced end portion, similarly heating and reducing the other end portion of the blank from said one side thereof by subjecting it to combined inward radial and lengthwise pressure between an interior die and an exterior recessed die, thereby producing the trunk of the T and a protuberance at one side of said trunk with the wall of the base portion of the protuberance of greater 45 thickness than the contiguous wall of the trunk, and forming the protuberance to final size and shape thereby producing the neck of the T joined to the trunk by a fillet of greater wall thickness than the trunk.

3. The method of producing a T, which comprises heating selected areas at one side of the end portions of a tubular metal blank to such a temperature that the metal thereof will readily flow when subjected to pressure, reducing the end portions relative to the central portion of the blank from said one side thereof by subjecting said end portions to combined inward radial and lengthwise pressure between interior dies and cooperating exterior dies interiorly recessed and shouldered effective for upsetting the wall of the blank at the areas of juncture between the central portion and said reduced end portions, thereby producing the trunk of the T and a protuberance at one side of said trunk with the wall of the base portion of the protuberance of greater thickness than the contiguous wall of the trunk, and forming the protuberance to final size and shape thereby producing the neck of the T joined to the trunk by a fillet of greater wall thickness than the trunk.

4. The method of producing a T, which comprises heating the end portions of a tubular metal blank to such a temperature that the metal thereof will readily flow when subjected to pressure, subjecting said end portions at one side

thereof to combined inward radial and lengthwise pressure effective for reducing the end portions of the blank relative to the central portion thereof and for upsetting the wall of the blank at the areas of juncture between the end portions and the central portion, thereby producing the trunk of the T and a protuberance at said one side of the trunk intermediate the end por-

tions thereof with the wall of the base portion of the protuberance of greater thickness than that of the trunk, and forming the protuberance to final size and shape thereby producing the neck 5 of the T joined to the trunk by a fillet of greater wall thickness than the trunk.

JAMES HALL TAYLOR.